

# UNITED STATES PATENT OFFICE.

JULIUS NEUMARK, OF NEW YORK, N. Y.

## PROCESS OF EXTRACTING TIN FROM TIN-PLATE WASTE.

SPECIFICATION forming part of Letters Patent No. 603,200, dated April 26, 1898.

Application filed September 10, 1897. Serial No. 651,243. (No specimens.)

*To all whom it may concern:*

Be it known that I, JULIUS NEUMARK, a citizen of the United States, and a resident of the city of New York, in the county and State 5 of New York, have invented a new and useful Process of Extracting Tin from Tin-Plate Waste, of which the following is a specification.

My invention consists of a novel electro-  
10 chemical process of treating tin scrap or waste to remove and recover the tin; and it has for its object to render the process regular in its operations and results and to make unnecessary the frequent renewal of the material 15 used as the electrolyte, as is required in operating the processes now in vogue. These prior processes consist, stated in general terms, in immersing the tin-scrap in an acid or an alkaline bath which will attack the tin, 20 especially when under the influence of an electric current passing through the bath, with the result that the tin is set free and deposited at the cathode of the electric circuit. Heretofore in such electrolytic processes several 25 very objectionable phenomena from a practical and economical point of view have developed. Thus after the electricity has acted for but a short time tin ceases to be set free and deposited, so that the process is short 30 lived. Furthermore, the baths offer great resistance to the electric currents after the process has been in operation a short time by reason of the tin salts which are taken up thereby, and if the strength of the current 35 be increased dangers arise and iron may be deposited. The result is that these processes have been irregular in their operation and required the frequent renewal of the electrolyte employed. These disturbances and objection- 40 able features are especially frequent and manifest when a caustic alkaline bath is employed as the electrolyte, for after the electric current has operated for a little while an alkaline tin salt is formed and becomes dis- 45 solved in the bath, with the result that the resistance of the electrolyte to the passage of the current rapidly increases, and the tin ceases to be set free and deposited at the cathode. At the same time a certain amount of 50 the caustic alkali is by the carbonic acid of the air converted into a carbonate and so be-

comes lost to the electrolytic process. If the electrolyte be replaced by a fresh bath after the process has ceased to operate satisfactorily, a large amount of tin is lost along with 55 the discarded electrolyte in the form of an alkali stannate, which, if the attempt should be made to recover it by evaporation, would be impure and worthless. Further, should it be attempted to force the process to successfully operate by largely increasing the voltage of the electric current new dangers arise, as oxygen and hydrogen are then set free and explosions become liable, especially where the process is carried on in closed vessels or re- 60 ceivers. These evils are entirely avoided by means of the process which I have invented and which I will now describe and by means of which the electrolyte is preserved as a 65 good conductor of electricity. 70

In describing my process I will assume that a bath of caustic soda is used as the electrolyte and the tin-scrap or the material from which the tin is to be recovered is placed in the bath and so connected as to become the 75 anode of the electric circuit. When the current is established, tin oxid is set free at the anode and is acted upon by the alkali in the bath, forming a sodium stannate, and at the same time metallic tin is set free at the cath- 80 ode. This action continues for a time; but finally the electrolyte bath becomes so charged with sodium stannate that the process ceases, as has been described, in a great measure or entirely. When this takes place, phosphoric 85 acid is added to the bath, with the result that a reaction takes place between the sodium stannate and the phosphoric acid—sodium phosphate, tin oxid, and water being formed—the tin oxid being precipitated. At the same 90 time whatever of sodium carbonate there may have been in the bath is converted into sodium phosphate. Sufficient calcium oxide is then added to the bath to react upon the sodium carbonate and convert it into sodium 95 phosphate, which is precipitated. At the same time sodium oxid is formed, and that in the presence of the water of the bath is converted into caustic soda, thus reviving the bath without withdrawing it, when the process of recovering the tin from the tin-waste 100 may be continued. The tin oxid which is

first precipitated is removed from the bath and the tin recovered mechanically, as by the well-known melting process. The precipitated calcium phosphate is drawn off and may 5 be used either in the preparation of new quan-



The reaction above indicated takes place in the presence of sufficient water to form a bath.

Having thus described my invention, what I claim, and desire to secure by Letters Patent, is—

1. The process of regenerating an alkaline electrolyte charged with salts of tin, which consists in adding phosphoric acid to the electrolyte and, after the reaction which takes 20 place is complete, adding calcium oxid to the electrolyte, substantially as and for the purposes hereinbefore set forth.

2. The herein-described process of recovering tin from tin-waste and the like, which consists in subjecting the tin-waste to the 25 joint action of a current of electricity, and a

ties of phosphoric acid in the well-known manner or as a fertilizer.

The process, so far as my invention is concerned, is indicated by the following equation, viz:

10

bath consisting of a solution of caustic alkali, until the recovery of the tin is retarded or ceases, and the bath becomes charged with tin salts; then adding phosphoric acid to the 30 bath, causing a precipitation of tin oxid; then adding calcium oxid to the bath, causing a precipitation of calcium phosphate, and removing the precipitates of such reactions, substantially as and for the purposes hereinbefore set forth.

In testimony whereof I have hereunto set my hand this 9th day of September, 1897.

JULIUS NEUMARK.

Witnesses:

ALFRED P. W. SEAMAN,  
RALPH H. HOLLAND.